

UNITED STATES PATENT OFFICE

**2,672,448**

# TRANSFORMER OIL CONTAINING A TERTIARY ALKYL PHENOL ANTIOXIDANT AND A DIHYDROXY ANTHRAQUINONE AS A SYNERGIST FOR THE ANTIOXIDANT

Charles D. Newnan, San Pablo, and Neal W. Furby, Berkeley, Calif., assignors to California Research Corporation, San Francisco, Calif., a corporation of Delaware

**No Drawing. Application September 27, 1952,  
Serial No. 311,944**

**11 Claims. (Cl. 252—64)**

1

This invention relates to the stabilization of lubricating oil compositions intended for use in the service of transformer oils, turbine oils, and the like. More particularly, this invention pertains to mineral oil compositions useful as transformer oils, wherein the antioxidation characteristics of the antioxidant present in the composition (e. g., 2,6-di-tertiary butyl-4-methyl phenol) have been enhanced by the presence of hydroxyanthraquinone compounds (e. g., quinizarin).

This patent application is a continuation-in-part of Newnan-Furby application Serial No. 159,141, filed April 29, 1950, now abandoned.

The effectiveness of transformer oils as insulating oils is materially reduced by the oxidation products (i. e., the acid products) formed. Furthermore, these acid products gradually attack the insulation on the wires of the transformer system, leaving the wires partially exposed to the oil, which oil then serves as a transmitter of current instead of an inhibitor of current. In the turbine oils the oxidation products (i. e., the acid sludges) corrode the bearings and other parts of the turbine system and clog the oil lines, etc.

It is a tremendous advantage in transformer, turbine, and like systems, to use the oils of sufficient oxidation stability to permit their use over long periods of time without being changed. Not only is it desirable to have transformer oils and the like highly resistant to oxidation, but it is also a desired feature of the transformer oils and the like that the viscosity index be high; that is, that only small changes in viscosity occur with large changes in temperature. Thus, in order to obtain oils of high viscosity index, the base oils are subjected to such effective methods of refining as selective solvent extraction processes wherein the lower viscosity index hydrocarbons are selectively dissolved. Selective solvent refining processes concentrate in one fraction, usually the undissolved oil fraction, those compounds of a "paraffinic" nature which show a smaller change in viscosity upon change in temperature. However, highly refined oils have smaller amounts of naturally occurring oxidation inhibitors present in the oils than do less refined oils. That is, naturally occurring inhibitors have been removed at least to an extent which materially reduces the oxidation stability of the oil when used as transformer oils and as turbine oils.

When oxidation inhibitors are added to highly refined oils and oils which are not so highly refined, it is found that the highly refined oils are more responsive to the oxidation inhibitors: that is,

2  
is, when the oxidation inhibitors of this invention are incorporated in so-called over-refined oils, a greater resistance to oxidation is obtained than when the oxidation inhibitors are used in conjunction with a less refined lubricating oil.

In attempting to increase the oxidation stability of transformer and turbine oils, known oxidation inhibitors (e. g., 2,6-di-tertiary butyl-4-methyl phenol) were incorporated therein, and, 10 as expected, the resulting compounded oils were more resistant to oxidation than the base oils containing no inhibitors. However, it was not to be expected that the oxidation stability of the oil thus compounded with oxidation inhibitors 15 could be increased still further by adding thereto an agent which by itself is not an oxidation inhibitor.

It is an outstanding feature of this invention that the oxidation stability of a lubricating oil compounded with an oxidation inhibitor is materially increased by adding thereto an agent not known as an oxidation inhibitor which agent asserts synergistic effects in combination with the oxidation inhibitors of this invention.

25 It is an object of this invention to incorporate in mineral oils containing oxidation inhibitors an agent exhibiting a marked synergistic effect on certain oxidation inhibitors.

It has been discovered that highly oxidation  
resistant lubricating oil compositions may be  
prepared by incorporating hydroxy anthra-  
quinones in lubricating oil compositions con-  
taining phenyl hydroxy compounds as oxidation  
inhibitors.

The hydroxy anthraquinones of this invention include anthraquinones containing two hydroxyl groups on the ring, such as exemplified by alizarin (1,2-dihydroxy anthraquinone), quinizarin (1,4-dihydroxy anthraquinone), anthra-ruffin (1,5-dihydroxy anthraquinone), chrysazin (1,8-dihydroxy anthraquinone), xanthopurpurin (1,3-dihydroxy anthraquinone), hystazin (2,3-dihydroxy anthraquinone), isoanthrafavinic acid (2,7-dihydroxy anthraquinone), etc.

45 The anthraquinones forming a part of the composition of this invention also include anthraquinones containing alkyl groups having from 1 to about 18 carbon atoms. These alkyl-substituted anthraquinones include 3-butyl-1,2-dihydroxy anthraquinone, 3-penta-1,2-dihydroxy anthraquinone, 4-hexyl-1,2-dihydroxy anthraquinone, 3-octyl-1,2-dihydroxy anthraquinone, 3-decyl-1,2-dihydroxy anthraquinone, 3-hexadecyl-1,2-dihydroxy anthraquinone, 3-octadecyl-1,2-dihydroxy anthraquinone, 2-butyl-55 1,3-dihydroxy anthraquinone, 2-butyl-1,3-dihydroxy

droxy anthraquinone, 2-butyl-1,4-dihydroxy anthraquinone, 2-hexyl-1,4-dihydroxy anthraquinone, 2-octyl-1,4-dihydroxy anthraquinone, 2-decyl-1,4-dihydroxy anthraquinone, 2-hexadecyl-1,4-dihydroxy anthraquinone, 2-octadecyl-1,4-dihydroxy anthraquinone, 2-eicosyl-1,4-dihydroxy anthraquinone, 2-triacontyl-1,4-dihydroxy anthraquinone, 2-nonyl-1,4-dihydroxy anthraquinone, 2-methyl-1,4-dihydroxy anthraquinone, 2-ethyl-1,4-dihydroxy anthraquinone, 2-methyl-1,5-dihydroxy anthraquinone, 2-octyl-1,5-dihydroxy anthraquinone, 2-nonyl-1,5-dihydroxy anthraquinone, 2-octadecyl-1,5-dihydroxy anthraquinone, 2-triacontyl-1,5-dihydroxy anthraquinone, etc. The 1,4-dihydroxy anthraquinones and the 1,5-dihydroxy anthraquinones are especially preferred because these dihydroxy anthraquinones are more effective in increasing the antioxidation effects of the phenyl hydroxy compounds as oxidation inhibitors of this invention.

Oxidation inhibitors which are contemplated by this invention to be used in viscous oil compositions in combination with the dihydroxy anthraquinones are the phenyl hydroxy compounds containing at least one hydroxyl group. That is, the oxidation inhibitors included herein are phenyl hydroxy (hydroxy phenyl) compounds containing one or more hydroxyl groups on the ring, preferably only one hydroxyl group on the ring.

When the phenyl hydroxy compound contains only one hydroxyl group, there can be from 1 to 5 alkyl groups present in the compound, the alkyl groups containing a total of from 3 to about 20 carbon atoms. However, it is preferred that there be three alkyl groups present, at least one of the alkyl groups being a tertiary alkyl group. It is especially preferred to use phenyl hydroxy compounds containing only one hydroxyl group and containing three alkyl groups, two of which alkyl groups are tertiary alkyl groups, particularly tertiary butyl groups.

Examples of the various phenyl hydroxy compounds which are included in the present invention are: monotertiary butyl-meta-cresol, 2,6-ditertiary butyl-4-methyl phenol, 2,4-ditertiary butyl-6-methyl phenol, 2,4,6-trimethyl phenol, 2,4,6-tritertiary butyl phenol, catechol, p-tertiary butyl catechol, resorcinol, 2-pentadecyl hydroquinone, etc.

The term "alkyl" as used herein means a saturated or unsaturated monovalent hydrocarbon radical; for example, methyl, ethyl, ethenyl, propyl, propenyl, tertiary butyl, secondary butyl, octenyl, pentenyl, decyl, decenyl, dodecyl, dodecyl, hexadecyl, heptadecyl, etc.

The mineral oil constituents of the lubricating oil composition include such base oils as naphthenic base oil, paraffin base, and mixed base mineral oils, other hydrocarbon lubricants, e. g., lubricating oil derived from coal products, and synthetic oils, e. g., alkylene polymers (such as polymers of propene, butene, etc., and mixtures thereof), alkylene oxide-type polymers (e. g., propene oxide polymers) and derivatives, including alkylene oxide polymers prepared by polymerizing alkylene oxides, e. g., propene oxide, in the presence of water or alcohol, e. g., ethyl alcohol, and esters of alkylene oxide-type polymers, e. g., acetylated propene oxide polymers prepared by acetylating propene oxide polymers containing hydroxyl groups.

Other synthetic oils include dicarboxylic acid

esters, polyesters, esters of polyhydric alcohols, and liquid esters of acids of phosphorus.

Synthetic oils of the dicarboxylic acid ester-type include those which are prepared by esterifying such dicarboxylic acids as adipic acid, azelaic acid, suberic acid, sebacic acid, alkenyl succinic acid, fumaric acid, maleic acid, etc., with alcohols such as butyl alcohol, amyl alcohol, hexyl alcohol, heptyl alcohol, 2-ethylhexyl alcohol, dodecyl alcohol, pentaerythritol, hexamethylene glycol, etc. Examples of dicarboxylic acid ester synthetic oils include dibutyl adipate, dihexyl adipate, di-2-ethylhexyl sebacate, condensation products of hexamethylene glycol and adipic acid, etc. Other synthetic oils include esters of polyhydric alcohols, e. g., pentaerythritol tetracaprate.

Synthetic oils of the type of liquid esters of acids of phosphorus include the esters of phosphoric acid, e. g., tricresyl phosphate; the esters of phosphonic acid, e. g., diethyl ester of decane phosphonic acid.

The oxidation inhibitors (i. e., the phenyl hydroxy compounds) which are present in the lubricating oil composition of this invention may be present in amounts from about 0.01% to about 3.0% by weight of the final composition, that is, an amount sufficient to increase the resistance of the lubricating oil composition to oxidation. It is preferred to use from about 0.1% to about 1.0% by weight, based on the finished composition.

The hydroxy anthraquinones of this invention (e. g., quinizarin) may be present in the final mineral oil composition in amounts from about 0.002% to about 1.0% by weight of the final composition. It is preferred to use an amount sufficient to enhance the oxidation inhibiting characteristics of the phenyl hydroxy compound, preferably from about 0.01% to about 0.1%.

In certain instances (for example, for shipping purposes) it is more preferable to prepare lubricating oil concentrates of the additives of this invention. That is, the phenyl hydroxy compounds of this invention can be present in lubricating oil compositions in amounts as great as 50% by weight of the final composition. The hydroxy anthraquinones can be present in such amounts as permitted by their solubility in the base oil, which, in some instances, is more than 1% and in other instances is less than 1%, even less than 0.5% by weight.

It was wholly unexpected that the hydroxy anthraquinones (e. g., quinizarin) would exert such synergistic effects upon the lubricating oil oxidation inhibitors (i. e., the phenyl hydroxy compounds). Nowhere would anyone expect to find such synergistic effects as disclosed herein by the addition of a synergist (i. e., a hydroxy anthraquinone) as a secondary agent to a lubricating oil composition containing additives which are known to inhibit oxidation, particularly to find these antioxidation properties enhanced so tremendously by the addition of a secondary agent which in itself has relatively no effect in inhibiting oxidation in a lubricating oil. It is well known in the art that the phenyl hydroxy compounds are remarkable oxidation inhibitors; but it is entirely new to discover this effect of the hydroxy anthraquinones on the oxidation inhibiting effects of the phenyl hydroxy compounds. Obviously, it is not merely an additive effect which is obtained between the combinations of the known oxidation inhibitor in the lubricating oil and the hydroxy anthraquinone be-

cause the hydroxy anthraquinones in themselves are practically ineffective in inhibiting the oxidation of lubricating oil compositions.

In the table hereinbelow, data are presented to show the synergistic effects obtained by testing the compositions of additives in a lubricating oil under severe conditions. In order to test effectively the compositions of this invention, a more drastic test was devised than is normally used in evaluating transformer oils and the like. This test has been called the California Research Transformer Oil Stability Test. The test is run as follows:

A 300 gram sample to be tested is placed in a glass tube which is set in an oil bath at 250° F. Oxidation catalysts, i. e., 112½ square centimeters of medium silicon transformer iron (such as U. S. S. Trancor 72) and 450 square centimeters of No. 14 gauge ASTM electrolytic copper wire are inserted in the tube. Oxygen is bubbled through the test sample at a rate of 3 liters per hour until the test sample has an acid number of 1.0 (milligrams of KOH per gram sample of oil). The number of hours required for the sample to show an acid number of 1.0 is known as the "test life" of the sample.

The data presented in Table I will serve to illustrate the nature of the results that were obtained in accordance with the present invention.

TABLE I

*Quinizarin in a mineral oil containing  
ditertiary butyl-4-methyl phenol*

| Test No. | Base Oil | 2,6-Ditertiary Butyl-4-Methyl Phenol | Quinizarin | Test Life (Hours) |
|----------|----------|--------------------------------------|------------|-------------------|
| 1.       | (1)      |                                      |            |                   |
| 2.       | (1)      |                                      | 0.05       | 24                |
| 3.       | (1)      | 0.3                                  |            | 25                |
| 4.       | (1)      | 0.5                                  |            | 80                |
| 5.       | (1)      | 0.2                                  | 0.005      | 104               |
| 6.       | (1)      | 0.2                                  | 0.02       | 155               |
| 7.       | (1)      | 0.3                                  | 0.01       | 180               |
| 8.       | (2)      |                                      |            | 230               |
| 9.       | (2)      |                                      | 0.05       | 24                |
| 10.      | (2)      | 0.3                                  |            | 20                |
| 11.      | (2)      | 0.3                                  | 0.05       | 70                |
| 12.      | (3)      |                                      |            | 275               |
| 13.      | (3)      |                                      | 0.05       | 24                |
| 14.      | (3)      | 0.3                                  |            | 20                |
| 15.      | (3)      | 0.3                                  | 0.05       | 175               |
|          |          |                                      |            | 400               |

<sup>a</sup> A California solvent-refined naphthenic base oil having a viscosity of 58 SSU at 100° F., and having 90% unsulfonatable residue.

<sup>b</sup> The base oil of (1) which had been treated further to yield an oil having 95% unsulfonatable residue.

<sup>c</sup> The base oil of (1) which had been treated further to yield an oil having 98% unsulfonatable residue.

The data set forth hereinbelow in Table II were obtained when using nonyl quinizarin as the dihydroxy anthraquinone. The base oil used in obtaining the data of Table II was the same base oil (2) of Table I hereinabove.

TABLE II

*Nonyl quinizarin in a mineral oil containing  
0.3% 2,6-ditertiary butyl-4-methyl phenol*

| Test No. | Nonyl Quinizarin (Percent by Weight) | Test Life (Hours) |
|----------|--------------------------------------|-------------------|
| 16.      |                                      | 80                |
| 17.      | 0.005                                | 300               |
| 18.      | 0.01                                 | 290               |
| 19.      | 0.05                                 | 290               |
| 20.      | 0.10                                 | 300               |

The data set forth hereinbelow in Table III 75

show the effect of adding quinizarin as the hydroxy anthraquinone to a lubricating oil containing 0.3% by weight of monotertiary butyl metacresol.

TABLE III

| Test No. | Amt. of Phenyl Hydroxy Compound (Percent by Weight) | Amt. of Hydroxy Anthraquinone (Percent by Weight) | Test Life (Hours) |
|----------|-----------------------------------------------------|---------------------------------------------------|-------------------|
| 21.      |                                                     |                                                   | 24 (2)            |
| 22.      |                                                     | 0.05                                              | 25                |
| 23.      |                                                     | 0.3                                               | 30                |
| 24.      | 0.3                                                 | 0.05                                              | 155               |

These data show that hydroxy anthraquinones produce a synergistic effect in oils containing phenyl hydroxy compounds having one hydroxyl group and at least two alkyl groups attached to the ring.

The data of Table IV hereinbelow illustrate the effectiveness of other anthraquinones as synergists in enhancing the stability of oil compositions containing phenyl hydroxy compounds according to applicants' invention.

TABLE IV

| Test No. | Additive (percent by Weight)         |                            | Test Life (Hours) |
|----------|--------------------------------------|----------------------------|-------------------|
|          | 2,6-Ditertiary Butyl 4-Methyl Phenol | Hydroxy Anthraquinone Used |                   |
| 35       |                                      |                            |                   |
| 25.      |                                      |                            |                   |
| 26.      | 0.3                                  |                            | 24                |
| 27.      |                                      | 0.05                       | 80                |
| 28.      | 0.3                                  | 0.05                       | 25                |
| 29.      |                                      | 0.05                       | 315               |
| 30.      | 0.3                                  | 0.05                       | 20                |
| 31.      |                                      | 0.05                       | 300               |
| 32.      | 0.3                                  | 0.05                       | 20                |
|          |                                      |                            | 185               |

<sup>a</sup> 2-(3,5,5-trimethyl-1-hexyl) quinizarin prepared by the reaction of quinizarin and 3,5,5-trimethyl hexaldehyde in the presence of aqueous sodium hydroxide and sodium hyposulfite at 95° C.

<sup>b</sup> 1,6-dihydroxy anthraquinone.

<sup>c</sup> 1,8-dihydroxy anthraquinone.

A combination of additives of the present invention are used effectively not only in transformer oils, turbine oils and the like, but are also used effectively in hydraulic oils, ice machine oils, instrument oils, etc.

Other groups of additives may also be used in the oils in addition to the components of this invention. For example, in addition to the above-noted compounds, the lubricating oils may contain other agents such as pour point depressants, oiliness agents, extreme pressure agents, blooming agents, compounds for enhancing the viscosity index of hydrocarbon oils, grease-forming agents, peptizing agents, etc.

We claim:

1. A transformer oil consisting essentially of a major portion of a lubricating oil and a minor portion of a combination of a tertiary alkyl phenol antioxidant for said lubricating oil and a synergist for said antioxidant, said antioxidant being present in an amount sufficient to increase the resistance of said oil to oxidation, said synergist being a hydroxy anthraquinone selected from the group consisting of alizarin, quinizarin, anthrarufin, chrysazin, and 2-methyl-1,4-dihydroxy anthraquinone, said synergist being present in the proportion of about 0.002% to about 1.0% by weight of said transformer oil.
2. The transformer oil of claim 1 in which

the phenol is present in the proportion of about 0.01% to about 3% by weight of said transformer oil.

3. The transformer oil of claim 1 in which the tertiary alkyl phenol is a tertiary butyl phenol.

4. The transformer oil of claim 1 in which the tertiary alkyl phenol is a tertiary butyl phenol.

5. The transformer oil of claim 1 in which the tertiary alkyl phenol is 2,6-ditertiary butyl-4-methyl phenol and in which the synergist is quinizarin.

6. The composition of claim 1 in which the lubricating oil is a petroleum hydrocarbon lubricating oil.

7. The transformer oil of claim 1 in which the synergist is quinizarin.

8. The transformer oil of claim 1 in which the synergist is chrysazin.

9. The transformer oil of claim 1 in which the synergist is alizarin.

10. A transformer oil consisting essentially of a major portion of a lubricating oil and a minor portion of a combination of a tertiary alkyl

phenol antioxidant for said lubricating oil and a dihydroxy anthraquinone as a synergist for said antioxidant, said antioxidant being present in an amount sufficient to increase the resistance of said oil to oxidation and said dihydroxy anthraquinone being present in about 0.002% to about 1.0% by weight of said transformer oil.

11. The transformer oil composition of claim 10 wherein said dihydroxy anthraquinone is substituted with at least one alkyl group having up to about eighteen carbon atoms.

CHARLES D. NEWNAN.  
NEAL W. FURBY.

## References Cited in the file of this patent

## UNITED STATES PATENTS

| Number    | Name         | Date           |
|-----------|--------------|----------------|
| 2,016,648 | Orelup       | Oct. 8, 1935   |
| 2,053,421 | Burk et al.  | Sept. 8, 1936  |
| 2,214,443 | Varteressian | Sept. 10, 1940 |
| 2,225,533 | Dewey        | Dec. 17, 1940  |
| 2,261,888 | Rocchini     | Nov. 4, 1941   |